

## UNITED STATES PATENT OFFICE

MARTIN HAHN, OF BORITZ, NEAR RIESA-ON-THE-ELBE, GERMANY

## PROCESS FOR PRODUCING AN EXPLOSIVE

No Drawing. Application filed March 20, 1929, Serial No. 348,665, and in Germany January 31, 1929.

The object of the present invention is to produce an explosive which can normally be handled and transported without the slightest danger and which can be readily changed 5 constitutionally so as to form an easily ignited, powerful explosive.

This object is achieved according to the invention by dissolving lime in nitric acid, adding cellulose and water and drying the mass 10 thus obtained, further addition of a solution of lime in nitric acid and re-drying being subsequently effected in order to render the explosive ready for use.

The explosive may be prepared as follows: 15 Burnt lime or calcareous earth is dissolved in raw, odorless nitric acid so as to produce a clear, transparent fluid resembling petroleum jelly. This fluid is diluted with 1-5 parts of water according to the desired 20 explosive power and is then mixed with cellulose in the form of peat power, sawdust or the like, until a consistent mass is obtained. This mass is given any suitable form and dried. The substance thus obtained is in- 25 sensitive to shocks, pressure and friction, even when hand-warm, and can therefore be handled and transported with safety.

In order to render the substance ready for use, it is again mixed with fluid obtained as 30 above by dissolving lime in nitric acid and re-dried. The resulting susbtance will be highly explosive and can be ignited electrically or by means of a fuse. It can be employed for the generation of machine power, for rock 35 blasting and other purposes.

I claim:

A process for producing explosives consisting in dissolving lime in nitric acid, dilut- 40 ing the solution with water, adding cellulose to the mixture until a consistent mass is ob- tained, drying said mass, adding further solu- tion of lime in nitric acid to the dried mass, and re-drying it for use after such addition.

MARTIN HAHN.